

No. 740,099.

PATENTED SEPT. 29, 1903.

S. C. DAVIDSON.

BUILDING OR ROOFING BLOCK OR MATERIAL.

APPLICATION FILED OCT. 16, 1902.

NO MODEL.



Witnesses

G. Howard Walmsley.  
James C. Hodges

By

Silas C. Davidson,  
Adison G. O'Brien  
his  
Attorney

Inventor

## UNITED STATES PATENT OFFICE.

SILAS C. DAVIDSON, OF BIRMINGHAM, ALABAMA.

## BUILDING OR ROOFING BLOCK OR MATERIAL.

SPECIFICATION forming part of Letters Patent No. 740,099, dated September 29, 1903.

Application filed October 16, 1902. Serial No. 127,592. (No model.)

*To all whom it may concern:*

Be it known that I, SILAS C. DAVIDSON, a citizen of the United States of America, residing at Birmingham, in the county of Jefferson 5 and State of Alabama, have invented certain new and useful Improvements in Building or Roofing Blocks and Material, of which the following is a specification.

My invention relates to an improvement in 10 building and roofing blocks or material, the objects of which are to produce a building or roofing block or material which can be cheaply made, the ingredients of which are everywhere at hand, and which material or building-block is absolutely impervious to water and 15 hence will not freeze.

Other objects are to furnish a material 20 or building or roofing block which will remain unaffected by atmospheric heat, having 25 strength, durability, and elasticity, and which is practically fireproof.

Another object is the provision of a building 25 or roofing block which can be remolded, if desired, even after having been in use for years.

Another object is the formation of an ornamental or other face upon the building or roofing block during its manufacture.

In the accompanying drawings, Figure 1 is 30 a perspective view of a building or roofing block constructed in accordance with my invention, and Fig. 2 is a view in cross-section thereof.

The building or roofing blocks may be composed of any one or all of a variety of ingredients—such as common earth, dirt, gravel, clay, sand, cinders, ashes, clinkers, crushed rock, slag—which ingredient or ingredients are caused to adhere or cohere by means of 40 coal-tar, the latter being employed as a binding agent.

In proceeding with the manufacture of my improvement I saturate a quantity of common dirt or earth with enough coal-tar to form 45 a very stiff mixture or, in other words, to make the resultant mixture cohere. In commingling the above-named ingredients I heat the entire mixture to a point where it will blaze from its own heat—say at about 160°—50 stirring to thoroughly mix the ingredients while heating.

In practice I have found that about eighty-

five per cent. to ninety per cent. of earth or dirt will form a sufficiently cohesive mass when mixed with from ten per cent. to fifteen 55 per cent. of coal-tar. The resultant mixture is placed in the molds while hot and compressed with a pressure of about one hundred pounds to the square inch. This forms a very dense block which may be laid while hot, and 60 by so doing the blocks will cohere to one another without the use of mortar or other adhesive agent, thus forming a solid structure. It will be understood that the percentage of coal-tar or other binding agent—such as crude 65 coal-oil, asphalt, or pine-tar, which may also be utilized—varies with the filling or body material employed. The proportions given refer to common dirt or earth and coal-tar.

In many instances it is desirable to employ 70 an ornamental or colored face brick and in pursuance of this idea I proceed as follows: After obtaining the mixture as above set forth I fill the molds nearly full therewith and fill the remaining space in the molds 75 with a mixture comprising about seventy per cent. of sand or dirt, fifteen per cent. of any preferred coloring agent, and fifteen per cent. of hard rosin, which ingredients are heated and commingled in a suitable receptacle separate from that in which the body of the brick is mixed. The molds thus filled are placed under pressure, and as a result I produce a building or roofing block which is harder than the ordinary burned brick and 80 costs about one-half as much.

It will be noted that I use but a single binding agent in combination with any sort of dirt or earthy matter, that my invention is very simple, and that the building-blocks are 85 easily constructed.

I am aware that it is old to mold the material while hot, that it is old to unite the blocks so constructed with a mortar comprising the same ingredients as do the blocks, and 90 I am also aware that composition blocks have been formed of a number of binding agents combined with a number of ingredients forming the body thereof; but I am not aware of any patent wherein any single filling ingredient, such as common earth, has been formed into a brick by means of a single binding agent—such as coal-tar, for instance—nor am I aware 95 that with a brick so constructed has been 100

combined an ornamental or color face, as set forth.

It is evident that there is a wide range of choice of binding agents and fillers which 5 might be used, as herein set forth, and consequently I do not wish to limit myself to any particular ingredients. I attain the desired result by the use of any of the above-named ingredients by properly proportioning them 10 before molding into building or roofing blocks which are compressed and laid while hot, and being thus compressed at a time when they are much hotter than they will ever become by reason of sun or atmospheric heat I overcome the laws of contraction and expansion. 15

Having thus fully described my invention, what I claim as new, and desire to secure by Letters Patent, is—

1. A building and roofing block comprising 20 a body portion composed of a filling material, a binding agent, and a color face composed

of a mixture of hard rosin, common dirt and coloring means.

2. A building or roofing block, comprising a body portion consisting of earthy matter or 25 dirt and coal-tar and a face portion consisting of sand or dirt, rosin and coloring-matter.

3. A building or roofing block consisting of a body portion comprising eighty-five to ninety per cent. of earthy matter or dirt and 30 ten to fifteen per cent. of coal-tar and a face portion comprising about seventy per cent. of sand or dirt, about fifteen per cent. of coloring-matter and about fifteen per cent. of rosin. 35

In testimony whereof I have signed my name to this specification in the presence of two subscribing witnesses.

SILAS C. DAVIDSON.

Witnesses:

B. F. FITZPATRICK,  
J. E. CUNNINGHAM.